

Jan. 23, 1945.

R. J. GREGORY

2,367,939

PROCESS FOR PRODUCING NAMEPLATES AND THE LIKE

Filed Feb. 5, 1943



WITNESSES:

E. A. McElroy  
J. Shapoe

INVENTOR

Royal J. Gregory  
By  
Frank J. Savage  
ATTORNEY

## UNITED STATES PATENT OFFICE

2,367,939

PROCESS FOR PRODUCING NAME PLATES  
AND THE LIKE

Royal J. Gregory, Elkridge, Md., assignor to Westinghouse Electric & Manufacturing Company, East Pittsburgh, Pa., a corporation of Pennsylvania

Application February 5, 1943, Serial No. 474,888

4 Claims. (Cl. 41—42)

This invention relates to ferrous metal nameplates and the like, and more particularly to a process for so applying protective organic finishes to ferrous metal sheets that the protective finish functions both to produce predetermined markings and to provide for good corrosion protection for the metal.

In applying organic finishes to ferrous metal in sheet form in producing nameplates, indicia and other members of similar nature, the problem of securing a good corrosion-resistant coating on the ferrous metal is as important as securing a clear and legible marking design or indicia. It has not been economical or easily feasible to combine a high degree of legibility in markings consisting of organic finishes with good surface coverage. In order to secure good coverage of the surfaces of the ferrous metal sheet, it is a requirement that any protective finish applied cover the metal surface as completely as possible. In order to secure a sharp and easily legible marking, it is generally necessary to apply organic finishes in such a fashion that there is no overlapping of the finishes. Obviously, it is difficult to meet this last requirement and still provide for as complete a coverage as possible.

The object of this invention is to provide for so applying protective organic finishes of different color to ferrous metal plates as to provide for predetermined legible markings while furnishing a high degree of corrosion protection to the metal.

Other objects of the invention will in part be obvious and will in part appear hereinafter.

For a fuller understanding of the nature and objects of this invention, reference should be had to the figure of the drawing showing schematically the sequence of steps necessary to produce the article of this invention.

Heretofore in producing nameplates and the like, it has been customary to use as a base a metal which is inherently corrosion-resistant. Such metals as Monel metal, stainless steel, aluminum, copper and brass have been selected for substantially all applications requiring nameplates and the like. According to this invention, less expensive and more easily obtainable metals have been found to produce highly satisfactory nameplates which will meet all the requirements for which more expensive base metals are employed.

In practicing this invention, mild steel sheets, for example, cold rolled steel, or clean hot rolled steel sheet, or in some cases cast iron plates, may be satisfactorily employed. The ferrous metal is

initially subjected to cleaning operations to remove grease and all surface dirt. For this purpose, wire brushing, sand blasting or acid pickling, followed by degreasing in a solvent vapor apparatus may be followed as is known to those skilled in the art. In some cases, anodic cleaning in an alkaline bath will produce surfaces of the requisite cleanliness.

In order to illustrate the practice of the invention, reference should be had to the figure of the drawing in which the step A illustrates a steel sheet 10 upon which it is desired to produce the marking or indicia "W" 12 in a protective finish of one color, for example, a black enamel, and a ground finish 14 of a contrasting color, for example, a white enamel.

In order to produce the marking on the clean steel sheet, the surface is initially coated with a layer of photo-sensitive emulsion 16 applied to one entire surface thereof. In case the sheet 10 is of such dimensions and the desired marking is only a small part thereof, it may be feasible to apply the emulsion to the small area at which the marking is to be produced. The photo-sensitive emulsion is of such a nature that, when subjected to photo-printing, certain portions of the emulsion may be removed, whereas other portions are rendered relatively non-removable and adhere to the surface of the sheet. By photo-printing a predetermined marking, pattern or design on the emulsion, the emulsion is rendered selectively removable at predetermined portions.

As shown at A, a "W" has been photo-printed on the emulsion. Upon removing the emulsion at these portions, generally by washing with water or some other suitable solvent, the bare metal surface is exposed in a predetermined pattern corresponding to the photo-print. The exposed metal can then be etched in the normal way, for example, in hydrochloric acid. As shown in step B of the drawing, the etched portion 18, which is a greatly enlarged section along B—B in step A, has been selectively etched by an acid leaving the surface 20 in relief. Etched depression 18 is of a depth such that it corresponds to the customary thickness of a coating of protective organic finish. However, the depth of etch may be varied within desired limits.

Subsequently, the emulsion 16 is removed from the surface of the plate 10 by applying a solvent therefor, for example, a mixture of nitric acid and hydrochloric acid. The upper surface of plate 10 as shown in step C carries an etched marking corresponding to that desired.

For some purposes of the invention, the plate

10 in step C may be treated with rust-proofing substances in order to confer on the ferrous metal an increased corrosion-resistance. For instance, phosphate solutions may be applied thereto in order to render the metal more rust-resisting. In some cases, the ferrous metal may be plated with a coating of zinc and the zinc subjected to a phosphate treatment to render any subsequently applied organic finish adherent thereto. In applying such rust-proofing coatings to the sheet 10, it is necessary that the coating be of substantially uniform thickness whereby a depression 18 corresponding to the etched marking may be maintained relative to the general relief 20 of the surface of the sheet.

15 The entire surface of the steel sheet 10, with or without rust-proofing treatment, is painted with a coating of protective organic finish of substantially uniform thickness within the etched depression 18 and on the relief 20. The back of the steel plate may be similarly painted, if it be desired. Spray painting is a satisfactory method of applying the finish. As shown at step D, the surface 20 and the etched depression 18 are now provided with a coating, for example, of white enamel 22, so that the enamel surface 26 in the etched depression 18 is below the enamel surface 24 as applied to the relief 20. The white enamel or any other protective organic finish is baked or dried until it is of a sufficient hardness.

20 In producing excellent nameplates, heat setting or polymerizing urea aldehyde, glycerophthalate or melamine resin enamels have been found to be quite satisfactory due to their gloss and other characteristics. Such enamels need be baked at a temperature of 400° F. for about fifteen minutes to produce a good finish. In some cases, radiant heat may be employed to dry the enamel 22.

25 The steel plate 10 with the baked or dried white enamel coating 22 is coated with a lithograph ink or its equivalent applied only to the relief surface 24 of the white enamel by means of a roller. As is illustrated at step E in the drawing, the depressed surface 26 of the white enamel is not coated with the lithograph ink 28.

30 Lithograph ink suitable for the practice of this invention consists of a boiled linseed oil which has been heat treated at a high temperature to an exceedingly viscous state. Carbonaceous pigments are added and turpentine or other solvent to give a desirable viscosity. For the purpose of this invention, lithograph ink or an equivalent varnish or other coating composition that may be heat treated at a high baking temperature without becoming insoluble or evaporating or being destroyed, is preferred. It is desired that the lithograph ink or its equivalent be such that the ordinary protective organic finishes will bake hard and dry in an oven to a relatively insoluble state while the ink is still soluble. The sheet 10 at stage E is then sprayed or brushed or otherwise treated to deposit in depression 26 a protective organic finish of a differing or contrasting color to the white enamel 22. The entire surface may be sprayed in the case of small objects, while in large nameplates or other members the contrasting finish may be applied substantially within the etched grooves.

35 As illustrated at step F, a black baking enamel 30 has been applied to the depressed surface 26 with some overlap over the lithograph ink 28. The sheet 10 secured at step F is baked in an

oven at a temperature of 350° C. for fifteen minutes, in case a urea aldehyde type of enamel is employed. After baking, the sheet is cooled and dipped into a solvent for the lithograph ink. Stoddard solvent or naphtha may be employed as solvents for the lithograph ink. The lithograph ink dissolves readily in such solvent, and the overlapped portion of the black baking enamel 30 may be easily removed by wiping with a felt or other material. It will be found that a sharp line will be secured between the black enamel 28 and the white enamel 22, whereby a high degree of legibility is secured.

40 The nameplates may now be pierced for attaching holes or blanked if a plurality of separate nameplates have been produced on one sheet of steel. To protect the edges of the ferrous plate from corrosion after being punched or pierced, it may be desirable to apply a coating of transparent lacquer or other transparent coating 32 to the entire sheet 10. The transparent lacquer will afford increased protection to the markings. The nameplate or other member so produced may be put to use immediately after the transparent lacquer has been thoroughly dried. The nameplates may be employed both indoors and outdoors.

45 The nameplates produced by the practice of this invention are characterized by a high degree of corrosion-resistance and ability to withstand normal wear and tear since the organic finish has been so applied as to substantially cover all exposed surfaces. The indicia or markings have been so applied that their juncture is sharp and the legibility is high. It will be found that the resultant painted surfaces 22—30 of the nameplates are of substantially the same level whereby there is no tendency for the indicia to be selectively abraded, thereby tending to illegibility with wear.

50 Since certain obvious changes may be made in the above procedure and different embodiments of the invention can be made without departing from the scope thereof, it is intended that all matter contained in the above description shall be interpreted as illustrative and not in a limiting sense.

I claim as my invention:

1. The method of producing a steel sheet with protective surface finishes of different color applied thereto so as to produce predetermined markings thereon and to secure adequate corrosion resistance, comprising, in combination, applying to the surface of the steel sheet a photo-sensitive coating which when subjected to a photo-printing can be treated to selectively etch the surface of the steel sheet, photo-printing a predetermined marking on the photo-sensitive coating, subjecting the photo-printed coating to an etchant to etch the surface of the steel sheet, thereby producing a relief pattern, removing the photo-sensitive coating, applying to the entire surface of the steel sheet a ground coating of protective organic finish of a selected color, applying lithograph ink to the relief portion of the surface without filling in the etched portions, applying a second coating of an organic finish of a contrasting color to the ground coating color to the etched portions, the lithograph ink preventing bonding of the ground coating and the contrasting color coating upon the relief surfaces, and applying a solvent for the lithograph ink when the organic finishes have dried whereby to remove the lithograph ink and the portions of the second coating on the relief, thereby pro-

ducing a steel sheet with surfaces having predetermined markings of contrasting coloring thereon.

2. The method of producing a steel sheet with protective surface finishes of different color applied thereto so as to produce predetermined markings thereon and to secure adequate corrosion resistance, comprising, in combination, applying to the surface of the steel sheet a photo-sensitive coating which when subjected to a photo-printing can be treated to selectively etch the surface of the steel sheet, photo-printing a predetermined marking on the photo-sensitive coating, subjecting the photo-printed coating to an etchant to etch the surface of the steel sheet, thereby producing a relief pattern, removing the photo-sensitive coating, applying to the entire surface of the steel sheet a ground coating of protective organic finish of a selected color, applying lithograph ink to the relief portion of the surface without filling in the etched portions, applying a second coating of an organic finish of a contrasting color to the ground coating color to the etched portions to a level substantially of the level of the coated relief, the lithograph ink preventing bonding of the ground coating and the contrasting color coating upon the relief surfaces, and applying a solvent for the lithograph ink when the organic finishes have dried whereby to remove the lithograph ink and the portions of the second coating on the relief, thereby producing a steel sheet with surfaces having predetermined markings of contrasting color thereon.

3. The method of producing a steel sheet with protective surface finishes of different color applied thereto so as to produce predetermined markings thereon and to secure adequate corrosion resistance, comprising, in combination, applying to the surface of the steel sheet a photo-sensitive coating which when subjected to a photo-printing can be treated to selectively etch the surface of the steel sheet, photo-printing a predetermined marking on the photo-sensitive coating, subjecting the photo-printed coating to an etchant to etch the surface of the steel sheet to a depth substantially equal to the thickness of a coating of organic finish, thereby producing a relief pattern, removing the photo-sen-

sitive coating, applying to the entire surface of the steel sheet a ground coating of protective organic finish of a selected color, applying lithograph ink to the relief portion of the surface without filling in the etched portions, applying a second coating of an organic finish of a contrasting color to the ground coating color to the etched portions to a level substantially of the level of the coated relief, the lithograph ink preventing bonding of the ground coating and the contrasting color coating upon the relief surfaces, and applying a solvent for the lithograph ink when the organic finishes have dried whereby to remove the lithograph ink and the portions of the second coating on the relief, thereby producing a steel sheet with surfaces having predetermined markings of contrasting color thereon.

4. The method of producing a ferrous sheet with protective surface finishes thereon of different color applied thereto so as to produce markings and to secure adequate corrosion resistance, comprising, in combination, applying to the surface of the ferrous sheet a photo-sensitive coating which when subjected to photo-printing can be treated with an etchant to selectively etch the surface of the ferrous sheet, photo-printing a predetermined marking on the photo-sensitive coating, applying an etchant to etched portions of the ferrous sheet thereby producing a relief pattern, removing the photo-sensitive coating, applying a substance for imparting a corrosion-resisting surface to the ferrous sheet without impairing the relief pattern, applying to the entire surface of the ferrous sheet a substantially uniformly thick coating of a protective organic finish of a selected color, applying a lithograph ink to the relief portions only, applying a second organic finish coating of a different color than the first coating of organic finish to the etched portions, the lithograph ink preventing adherence or bonding of the second coating to the first coating upon the relief surfaces, treating the ferrous sheet to dry the organic finishes, subjecting the sheet to a solvent for the lithograph ink to remove the lithograph enamel and that portion of the second coating upon the relief surfaces, and applying a transparent protective finish over the markings so produced.

ROYAL J. GREGORY.